

## UNITED STATES PATENT OFFICE

2,500,912

## METHOD OF MAKING ALLOYS

John J. McLaughlin, Chicago, Ill., assignor to  
Crimora Research and Development Corpora-  
tion, Crimora, Va., a corporation of Virginia

No Drawing. Application December 20, 1944,  
Serial No. 569,097

## 1 Claim. (Cl. 75—27)

1

This invention relates to a method of making alloys, and has particular reference to the introduction of manganese into magnesium or magnesium alloys having a relatively low melting point.

One aim of the invention is to reduce the time required to perform the alloying operation.

Another aim is to substantially reduce the amount of external heat that is required to fuse the metals and produce a homogeneous alloy.

Still another aim is to employ heat resulting from an exothermic reaction, for melting the manganese used in making the desired alloy.

A further aim is to form the manganese into a mass or briquette with material, capable of causing an exothermic reaction, for producing sufficient heat to melt the manganese, to the end that it will fuse and be mixed thoroughly with the other components of the desired alloy.

Other aims and objects of the invention will appear in the following description.

The method applies principally to the production of alloys containing high percentages of magnesium, which have many desirable properties and useful purposes. In accordance with the invention, such an alloy can be formed by first melting a batch of magnesium or magnesium alloy and then adding manganese, in the form of briquettes, which also contain materials capable of producing an exothermic reaction that is started when the briquettes are immersed in and subjected to the temperature of the molten magnesium.

The briquettes are preferably formed by mixing finely divided or powdered manganese, such as is obtained by the electrolytic recovery process, with a powdered oxide of manganese, such as  $MnO_2$ , and powdered magnesium. Other oxides of manganese, such as  $MnO$ , and  $Mn_2O_3$  and  $Mn_3O_4$  can be used. Also, aluminum in powdered form can be used as a substitute for or in combination with magnesium. The oxide of manganese and the magnesium or aluminum are used to effect the exothermic reaction, the amounts depending upon the rate at which it is desired that the reaction shall take place and other factors, such as the desired, final temperature of the fused batch.

When manganese dioxide and magnesium are used, the magnesium content should be more than half of the oxide content, so that no manganese oxide ( $MnO$ ) will be formed and cause a corresponding loss of manganese. If aluminum is used instead of magnesium and it is desired that no appreciable amount be added to the melt, the aluminum should be stoichiometrically equiv-

alent to the  $MnO_2$  or other oxidizing agent used. In either case, the amount of oxidizing agent employed should be sufficient to provide available oxygen of from 1% to 5% of the weight of the briquettes, employing either aluminum or magnesium, or both.

The constituents of the briquettes should be thoroughly mixed and then pressed sufficiently to provide a density sufficient to make them sink readily in the molten bath of magnesium. For example, a pressure of the order of 10,000 pounds per square inch should be used to compress manganese briquettes. The  $MnO_2$  should be as free from silica as possible, since the presence of silicon is detrimental to the efficient alloying of manganese with magnesium. If desired, a pure manganese dioxide can be used. It can be prepared from electrolytic manganese by dissolving nitric acid and decomposing the nitrate to produce a gray, hard dense manganese dioxide.

When briquettes are prepared in which about 5% to nearly 10% of the total manganese present is in the form of  $MnO_2$ , the balance existing in the form of manganese metal, and such briquettes are introduced into a melted mass comprising principally magnesium, a metal efficiency of 90% or better may be obtained. Total percentages of manganese of the order of about 0.5% may be readily introduced into magnesium in this manner; but greatly increased amounts, up to 5% may be added easily, if desired. The briquettes may be prepared in any suitable size to facilitate handling. Briquettes of general disc shape three inches in diameter and approximately one inch in thickness have been found suitable for the purpose.

As an example of the process, manganese was fused with a 40 pound batch of magnesium alloy containing about 6% aluminum and 3% zinc. The 40 pound batch was melted in an iron pot under a chloride flux and heated to approximately 700° C. Approximately one-third of a pound of previously prepared briquettes were introduced, said briquettes containing 25% powdered magnesium, 5% manganese dioxide and 70% metallic manganese of 65 mesh. The briquettes sank into the molten metal and dissolved with a vigorous convective motion of the molten metal but with no excessive spitting or boiling. The mass was permitted to cool to allow separation of impurities, such as iron, and it was found, on analysis, that the manganese content of the alloy was approximately .56%, which corresponded to more than 90% of the total added manganese.

The process may be practiced in other ways

and with other percentages of manganese and briquettes having percentages of materials other than those given in the specific example. When the process was carried on in the same manner as given in the example, but employing briquettes containing 10% of manganese dioxide, the mass boiled rather violently but in a controlled manner. In an open vessel, the reaction was impractically violent when the briquettes contained 20% manganese dioxide and quite an incendiary effect was obtained when the briquettes contained as much as 50% manganese dioxide.

The method may be carried out also by introducing the desired amount of manganese, for example, from 0.1% to 5%, into pure magnesium, the total weight of briquettes being calculated to the proper amount of manganese, and the resulting product then alloyed with other elements such as zinc, aluminum, copper and the like, by introducing the same in the manner customarily used in making magnesium alloys. It has been found, however, that if the briquettes are added to the otherwise completed alloy, iron and other impurities can be removed more effectively than when the manganese is added to the magnesium and the other alloying elements subsequently added.

Other oxidizers than  $MnO_2$  or oxides of manganese can be used. For example, nitrates, especially sodium and potassium nitrate can be used. Also, it is contemplated that chlorates and perchlorates can be employed. If any chlorine is evolved it would tend to clean up the metal. In addition, permanganate and dichromate can be used. It is further contemplated that cerium metals can be used as a substitute for magnesium

or aluminum to react with the oxidizer for producing the exothermic reaction.

Since certain changes can be made without departing from the spirit and scope of this invention, it is intended that all matter contained in the description thereof shall be interpreted as illustrative and not in a limiting sense.

What is claimed is:

10 The method of adding manganese to an alloy of magnesium, zinc and aluminum containing a high percentage of magnesium, the steps which comprise melting the alloy; and introducing into the molten bath exothermic strongly coherent briquettes containing from 5% to 10% manganese dioxide, approximately 25% magnesium, and the balance, manganese powder.

JOHN J. McLAUGHLIN.

#### REFERENCES CITED

20 The following references are of record in the file of this patent:

#### UNITED STATES PATENTS

|    | Number    | Name                  | Date          |
|----|-----------|-----------------------|---------------|
| 25 | 778,345   | Weber -----           | Dec. 27, 1904 |
|    | 906,009   | Goldschmidt -----     | Dec. 8, 1908  |
|    | 2,250,687 | Zeppelin -----        | July 29, 1941 |
|    | 2,267,862 | Hanawalt et al. ----- | Dec. 30, 1941 |
|    | 2,337,314 | Deppeler -----        | Dec. 21, 1943 |

#### FOREIGN PATENTS

|    | Number  | Country             | Date          |
|----|---------|---------------------|---------------|
|    | 20,004  | Great Britain ----- | A. D. 1905    |
| 35 | 185,749 | Great Britain ----- | Sept. 7, 1922 |
|    | 115,655 | Australia -----     | July 31, 1942 |